

Jan. 16, 1940.

C. G. YOUNG

2,187,294

PROCESS FOR STIFFENING PAPER

Filed Jan. 31, 1938



Inventor  
Clare G. Young  
by *J. Hutchinson Young & Co.* attys.

## UNITED STATES PATENT OFFICE

2,187,294

## PROCESS FOR STIFFENING PAPER

Clare G. Young, Winnipeg, Manitoba, Canada

Application January 31, 1938, Serial No. 187,981

## 1 Claim. (Cl. 18—56)

My invention relates to improvements in processes for stiffening paper and other flexible manufactured material principally for the production of light-weight slats for Venetian blinds but also for the manufacture of cartons and other articles of manufacture.

An object of my invention is to provide means whereby flexible material such as paper, may be stiffened economically and rendered resistant to heat, water and the effects of sunshine.

A further object of my invention is to provide in a Venetian blind, slats manufactured by the process hereinafter to be described to which will be imparted additional stiffness by virtue of an arcuate or convex cross-sectional configuration.

With the above more important objects in view and such other minor objects as may appear as the specification proceeds, my invention consists essentially in the arrangement and construction of parts all as hereinafter more particularly described, reference being had to the accompanying drawing in which:

Figure 1 is a perspective illustration of my Venetian blind.

Figure 2 is a sectional representation of the process of die-pressing the slats forming my Venetian blind.

In the drawing like characters of reference indicate corresponding parts in the different figures.

The slats for Venetian blinds have hitherto been manufactured of various straight grained woods such for example as fir, Australian gum, ash and the like. These possess the comparative disadvantage in relation to the slats manufactured by the process hereinafter described, of being heavy and costly to manufacture as well as noisy when raised. Slats manufactured by my process, however, may be made for a small fraction of the cost of wooden slats, are considerably lighter in weight and do not produce the same amount of noise when being raised.

In the practical carrying out of my process for the treatment of flexible material in the manufacture of Venetian blind slats, I have found the best material to be red press paper which I cut to the length and width required, after which it is submerged for fifteen minutes in a vat containing a mixture of animal glue and cold water, the texture of the mixture being that obtained when one pound of such glue is mixed with one gallon of cold water.

A large number of sheets I cut to the necessary length and size are generally placed together in a vat containing the foregoing mixture,

after the fifteen minutes steep the soaked sheets are placed one by one upon a die 2, prior to being pressed as will later be described. Upon the bearing surface of the two dies between which the soaked sheets or slats are pressed, I take a sheet of board 3, cut to the length and width of the slats, the said board being coated on both sides with paraffin wax. I now place upon the board one of my sheets of soaked press paper and above this another wax covered board. The number of soaked press paper sheets which are each sandwiched between the wax covered boards may be considerable, the topmost sheet being covered also by a wax covered board against which the upper die 4 bears in the pressing operation.

As I have already stated, my slats are arcuate or convex in cross-sectional configuration and to obtain this shape I simply make use of a male and female die of a corresponding shape, these dies being suitably secured in a press 5 one below the other. It is immaterial whether the male or convex die is secured to the bed 6 of the press or whether the female or concave die is so secured, as the alternate sheets of press paper and wax covered board may be built up in the alternate arrangement already described upon either the female or the male die.

The glue impregnated sheets of press paper remain in the press for eight hours during which time the glue is forced well into the paper, the efficiency of this action being increased due to the fact that the sheets of press paper are curved in cross sections which has the effect of opening one side of the sheet while closing the other side. When taken out of the press, the glue impregnated sheets are slats of a hard and smooth surface and possess considerable rigidity in themselves, apart from the additional rigidity obtained through the cross-sectional curvature thereof. They are now placed upon dryers which further improve the finish.

When dry, the slats are painted with an application of oil paint of good quality and body whereupon they are ready to be formed into a Venetian blind 7.

It should be mentioned that immediately after being cut to shape and before being steeped in the vat of glue, I cut or punch out the necessary apertures through which the blind cord has to pass.

Finally, I would mention that although I have described my process of treatment of paper sheets for the manufacture of Venetian blind slats, I do not confine myself in the ambit of patent pro-

tection claimed to this article of manufacture alone since it is obvious that many articles of manufacture may be made with paper treated in the foregoing manner. Furthermore, I do not confine myself to the use of red press paper as other papers may be found equally suitable. Moreover, other flexible materials apart from paper may prove suitable such as textiles, felt and the like.

10 Since various modifications can be made in the above invention, and many apparently widely different embodiments of same, made within the scope of the claim without departing from the spirit and scope thereof, it is intended that all 15 matter contained in the accompanying specification shall be interpreted as illustrative only and not in a limiting sense and I desire only such limitations placed thereon as are specifically expressed in the accompanying claim.

20 What I claim as my invention is:

In the manufacture of convex Venetian blind slats, the process which consists in steeping strips of press paper previously cut into strips of the

desired length and width for approximately fifteen minutes in a solution of animal glue and water mixed in the proportion of approximately one pound of glue to one gallon of water, afterwards placing one of said strips upon a cardboard slat coated with paraffin wax, said slat having previously been placed upon a die, then superimposing alternate slats and strips upon the lowermost strip to a desired height so that a slat is at the apex of the pile so formed, then exerting pressure upon said strips and slats to squeeze the same together by means of a die in bearing engagement with the topmost slat, one of said dies being concave and the other convex to impart a convex cross-sectional configuration to 15 said strips and said slats, said strips and said slats being maintained in a state of pressure between said dies for a period of approximately eight hours during which period the said solution of animal glue and water will be forced into the 20 cells of said strips.

CLARE G. YOUNG.